

## UNITED STATES PATENT OFFICE

2,131,137

## WASHING PROCESS FOR TEXTILE MATERIALS

Ehrhart Franz, Leipzig, Germany

No Drawing. Application December 12, 1933,  
Serial No. 702,031. In Germany December 13,  
1932

1 Claim. (Cl. 87—5)

This invention relates to a washing process for raw, semimanufactured and finished textile materials.

The process according to the invention is suited particularly for cleaning very dirty textiles, containing pitch, tar, oil, wax, resins or color. As the process does not injure the materials, it can be applied also for cleaning sensitive animal and vegetable textiles including silk, hair and wool. 10 Since wool is particularly sensitive, the removal of pitch and suint offered the greatest difficulties hitherto to the known cleaning methods. The pitch referred to involves the colors used for marking animals to prevent the theft thereof and 15 comprising, as a rule, linseed oil, pitch, resins, asphalt, etc., usually mixed with pigments. Most marking colors contain red lead or colored earths. The suint, on the other hand, is a secretion of abnormally functioning sebaceous glands and in 20 most cases due to improper treatment of the animals, though it may also indicate degeneration. With respect to their chemical and physical behavior, the most essential constituents of suint are waxes. Both impurities are not removed by 25 normal washing employing soap and weak alkalies and resist even solvents used in the washing process. This can be understood if it is taken into consideration that resinified linseed oil, pitch, cumarone resins, etc. are very difficultly 30 soluble, or not at all, in the usually employed easily boiling organic solvents, whereas red lead, pigments and colored earths will not dissolve at all in such substances. In practical operation, it was therefore preferred hitherto to pick out by 35 hand all parts affected by pitch or suint and burn them whereby considerable losses of expensive materials were brought about. Pitchy impurities are found even in finished goods, such as felts for pianos, which had to be carefully supervised till 40 now to detect and remove the impure portions thereof.

The invention provides a process according to which impure textile materials are treated with high-boiling chemical compounds which saturate 45 the impurities, soak and partially dissolve them. Besides the water soluble organic, aliphatic, aromatic, hydroaromatic and heterocyclic amines, such as pyridine, ethylene diamine, ethanol amine, the class of aliphatic acids, whether true 50 or ester acids, was found to give special satisfaction. Acids of this group comprise the aliphatic substituted or non-substituted carboxylic acids having 12 and more carbon atoms and their derivatives, such as lauric acid, palmitic acid, 55 stearic acid, myristic acid, elaidic acid, oleic acid

and their dichloroderivative, as well as the esters of these acids, e. g., the aralkyl esters, glycol esters, glycerin esters, etc., all of which can be used like the acid salts thereof and related salts. Likewise, the substituted or non-substituted aliphatic sulfo acids, sulfamic acids of sulfur ester acids, possibly in the form of their sodium or potassium salts, may be used, such as stearic, palmitic, elaidic sulfo acids, the oleylaminooethane sulfo acid, the ricinoleic and diricinoleic 10 sulfo acids as well as the stearyl alcohol sulfuric acid, the oleylalcohol sulfuric acid and their esters and salts; if the compounds mentioned are not oily, they are used in concentrated aqueous solution. To this class belong also the sulfonated fats and oils like Turkey red oil and sulfonated tallow. The corresponding phosphoric acids or phosphoric acid esters may also be used, especially in the form of their acid salts or acid 15 esters. The compounds as such or in the form 20 of their concentrated aqueous solutions possess a high penetrating capacity, so that they penetrate the impurities, soften them and dissolve them partly. After this soaking step, the high-boiling 25 chemical compounds together with the impurities 30 are removed from the fibers, preferably and as much as possible by mechanical means, e. g., squeezing or hydroextracting, the remainder being suspended in the impurity or the most difficultly soluble parts thereof. The substances concerned 35 may themselves act as emulsifiers for aqueous suspensions like the sulfo acids, the sulfuric acid esters, the phosphoric acids and esters, and the acid salts and carbonates. Preferably, alkaline washing waters are used, which is absolutely necessary if free carboxylic acids have been employed, as the latter, unlike their salts, the soaps, possess only slight emulsifying properties. The impurities are thus removed from the 40 textiles and remain as suspension in water while the compounds used for soaking serve then as emulsifiers. To simplify the process the squeezed or hydro-extracted material may be placed directly in the usual washing liquors which are slightly alkaline and finish it together with the 45 normal stuff. The substances used for soaking can be recovered from the washing liquors either by salting out or adding mineral acids. The separated compound is purified in the usual way, possibly by filtration and then employed again 50 for soaking impurities of another lot according to the invention. Instead of homogeneous compounds, solutions or suspensions of the high-boiling chemical compounds mentioned may be applied.

The following examples serve to explain the invention without limiting it to the details stated therein.

*Example 1*

- 5 The wool rendered impure by sticky tips is first shortly washed, hydro-extracted and dried to remove sand and dirt and loose grease. In the milling vessel the wool is saturated at normal or slightly increased temperature with twice its 10 weight of commercial olein. After five to twenty hours, according to temperature, the impurities can be ground with the fingers. The excess olein is then removed by squeezing or hydro-extracting, and the wool placed in a weakly alkaline 15 washing bath wherein the washing process is completed in the usual manner at 50° C. By adding sulfuric acid to the washing water the olein can be recovered and used for the same process after having been purified by one of the customary methods, e. g. filtration.

*Example 2*

Sticky wool is saturated with pyridin and treated in cold or slightly heated water until the 25 pitch is softened and partly dissolved. The excess pyridin is then removed, and the wool washed with a weak soap solution. The same effect can be attained when employing oleyliminoethylene-iminoethylenedimethylamine.

*Example 3*

Wool containing waxlike suint and picked out of normally washed lots is saturated with Turkey red oil (50% quality), which requires about 2 or 3

times the weight of the wool. The wool is allowed to stand at 20° C. until the impurities can be crushed between the fingers, which is usually the case after 6 to 8 hours. The material is then squeezed whereupon the excess Turkey red 5 oil is removed by centrifuging and afterwards the wool added to the normal lots for taking part in the usual washing process. From the washing waters part of the oil can be recovered by the addition of common salt and used again for 10 the same purpose.

*Example 4*

Raw cotton containing resinous or color impurities is saturated with twice the amount of 15 ground nut oil acid. After the cotton has remained therein for 20 hours, it is squeezed and placed in a bath of 5% potash lye, whereupon it is hydro-extracted and washed in an alkaline 20 washing liquor until the washing process is completed.

I claim:—

The process of removing pitch from a textile material comprising steeping the material in a liquid higher fatty acid softener for pitch of a 25 quantity exceeding the material in weight until the pitch has become friable when the material is rubbed between fingers, removing so much of the acid as can be mechanically removed, rendering the remaining acid water-soluble by introducing an aqueous alkaline solution to saponify the same, and then washing off the saponified acid together with the pitch emulsified therein.

EHRHART FRANZ.